

April 22, 1941.

T. N. HOGLUND

2,239,386

METHOD OF PHOTOENGRAVING

Filed June 12, 1939



INVENTOR,  
BY Thorle N. Hoglund  
M. Talbert & Dick  
ATTORNEY.

## UNITED STATES PATENT OFFICE

2,239,386

## METHOD OF PHOTOENGRAVING

Thorle N. Hoglund, Des Moines, Iowa

Application June 12, 1939, Serial No. 278,635

4 Claims. (Cl. 95—5.7)

The principal object of my invention is to accomplish desired staging and drop-outs automatically in the process of photoengraving.

A further object of this invention is to provide a method wherein the plate, prior to the etching phase, is of a darker tone thereby making possible a deeper etching without loss of color values.

A still further object of my invention is to provide a method whereby the ordinary square highlight dot becomes an elongated rectangular one and a round shadow dot becomes an elliptical one.

A still further object of my invention is to provide a method wherein the highlight dots are etched faster than the highlight dots next in size, the middle tones are etched faster than the next darker tones, the darker tones are etched very slowly, and the next darker tones are substantially free of etching.

A still further object of my invention is to provide a method of photoengraving wherein the printing from the finished plate is capable of greater contrast.

A still further object of my invention is to provide an easy method of photoengraving that is rapid and economical and substantially eliminates hand staging.

Photoengraving is very old. The process, however, is very tedious and great care must be exercised. In most instances much hard work is necessary to increase etching of certain parts of the plate and to retard or to completely stop etching of certain other parts of the plate. Even the most experienced engraver, however, cannot completely control all tones in the etching and, to substantially overcome such difficulties, I have provided my method, which is more of an automatic method of obtaining the desired results.

The usual way of making an etching on a plate of copper, zinc or like is to sensitize the plate with a suitable solution, common in the trade, after which the sensitized face is subjected to light through a photographic half-tone negative. Obviously, the negative is an ordinary one containing the picture-impression of the subject matter to be placed on the plate. Where the light passes through the transparent and translucent parts of the negative, the sensitized coating on the plate will adhere to the plate. The balance of the sensitized coating can be washed away, thereby leaving parts of the metal plate exposed for etching. Any suitable etching solution may be used and after the plate has been subjected to such solution the image of the subject matter on the plate will be in relief, and obviously, the high

points of the relief will become the printing part of the plate when put into printing usage. However, it will be noted that by etching or continuing the etching, these printing surfaces or places where the sensitized solution adhered will become smaller and smaller resulting in too light and too flat tones. The reason for this is that the entire impression on the plate is in the form of dots and after the etching solution eats into the plate at the sides of the printing dots, it commences to eat on the side walls of the printing dots and undermine the high points from all sides, thereby making the dots or projections smaller and smaller. To prevent this in certain instances and to produce a finished plate of the desired printing contrasts, certain of these tones are painted in or staged to prevent graying out and then the plate is subjected again to the solution. This may be repeated many times in order to gain the desired result.

My method, however, is to eliminate such problems in photoengraving and I obtain a better impression on the sensitized coating of the plate and change the shape of the ordinary round shadow dot and ordinary square highlight dot. After the initial subjecting of the plate to light through a negative, I resensitize the plate and then subject it to a second exposure of light through the negative. The plate is then developed. This means two separate exposures before the plate is etched. The second exposure will provide darker tones and this means one can etch maximum depths without loss of color values. In making the second exposure, the negative is slightly shifted in position in order that it will not exactly register with the first impression. By this action, the square highlight dot becomes an elongated rectangular one and the round dot becomes an oval one.

Although the double exposure in itself has great advantages for deep etching in the usual manner, the shifting of the negative in the second exposure and the changing of the outline of the dots has great potentialities in the use of dragon's blood powder, etching ink, and the like. The use of dragon's blood powder, ink and like to retard the etching processes after the first etching bite, on certain dots or sections of a plate, are well known.

The significance of this phase, however, is due to the odd shape of my shadow and highlight dots. In my method, the etching powder is banked against the long sides of the elongated rectangular dots. This is done in the usual manner by brushing the powder forth and back,

thereby leaving the ends or short walls exposed for further etching in the highlights. The plate is heated to melt the powder as it becomes acid resistant. By this procedure, the elongated rectangular highlight dots will be eaten away from both ends, thereby making the same smaller and substantially square. This means that the highlight dots will be reduced, while the shadow dots will remain substantially as before. This is due to the fact that the finest shadow dot is 10 too fine to keep open in any part, and, therefore, etching has ceased. The sensitized coating or enamel on the plate is the same thickness on all dots and the larger dots are, therefore, not effected by the thickness of the enamel. On the 15 other hand, the small shadow dots are practically closed by the enamel. The part therefore left exposed for etching is a percentage relative to the size of the shadow dot. The smaller the dot, the less area for attack of the etching solution. This is because the smaller the shadow dots, the more they close up by enameling and powdering. Therefore, the highlight dots are etched faster than the dots next in size and the 20 middle tones are etching faster than the next 25 darker tones. Also, the next darker tones are etching very little and the dark tones not at all.

It should also be noted that the shadow dots which are elliptical will, by the use of powder banked along their small inner ends, be etched into a round dot, thereby making such shadow dots their original shape and size as if only one exposure had been made, but without loss of color due to a darker print. This means that 30 great depth has now been reached in the etching process and a dot which received but a very slight etch will now be closed and the other dots will close up in proportion to their size.

This leaves only the middle tones etching 40 slightly, leaving highlight dots receiving most of the etching.

Obviously, other effects may be obtained by powdering the plate in three directions or powder from each of the four directions. This procedure leaves a larger percentage of etching in 45 the highlights. The shadow dots remain the same as heretofore explained.

Fig. 1 of the drawing illustrates the step by step procedure of my method.

Certain changes may be made in my method of photoengraving without departing from the spirit and purpose of this invention, and it is my intention to cover in my claims any reasonable modification thereof.

I claim:

1. A method of photoengraving comprising, the preparing of the surface of a plate with a suitable sensitized covering, the placement of a screened half-tone negative forward of and on the sensitized face of said plate, the passing of 60 light rays through said negative, and on to the

sensitized face of said plate, the resensitizing of the face of said plate with a suitable sensitized covering, the replacement of the said negative forward of and on the sensitized face of said plate with the negative slightly shifted from its original position on said plate, the passing of light rays through said negative and on to the sensitized face of said plate, the washing of said plate and the etching of said plate with a suitable etching solution.

2. A method of photoengraving comprising, the preparing of the surface of a plate with a suitable sensitized covering, the placement of a screened half-tone negative on the sensitized face of said plate, the passing of light rays through said negative, and on to the sensitized face of said plate, the resensitizing of the face of said plate with a suitable sensitized covering, the replacement of the negative on the sensitized face of said plate, and slightly shifted in its position relative to its first position on said plate, the passing of light rays through said negative and on to the sensitized face of said plate, the washing of said plate and the etching of said plate with a suitable etching solution.

3. A method of photoengraving comprising, the preparing of the surface of a plate with a suitable sensitized covering, the placement of a screened half-tone negative on the face of said plate, the passing of light rays through said negative, and on to the sensitized face of said plate, the resensitizing of the face of said plate with a suitable sensitized covering, the replacement of the negative on the sensitized face of said plate, and slightly shifted in its position relative to its first position on said plate, the passing of light rays through said negative and on to the sensitized face of said plate, the washing of said plate and the etching of said plate with a suitable etching solution, the subjecting of the plate to an etching powder, and the re-subjecting of said plate to a suitable etching solution.

4. A method of photoengraving comprising, the preparing of the surface of a plate with a suitable sensitized covering, the placement of a screened half-tone negative on the face of said plate, the passing of light rays through said negative, and on to the sensitized face of said plate, the resensitizing of the face of said plate with a suitable sensitized covering, the replacement of the negative on the sensitized face of said plate, and slightly shifted in its position relative to its first position on said plate, the passing of light rays through said negative and on to the sensitized face of said plate, the washing of said plate and the etching of said plate with a suitable etching solution, the banking of the resultant dots with an etching powder from two directions, and a re-etching of said plate with a suitable etching solution.

THORIE N. HOGLUND.